

## 1

3,813,331

**DEMETALATION OF HYDROCARBON CHARGE STOCKS WITH MANGANESE NODULE CATALYST**  
Paul B. Weisz, Yardley, and Anthony J. Silvestri, Morrisville, Pa., assignors to Mobil Oil Corporation  
No Drawing. Continuation-in-part of application Ser. No. 100,931, Dec. 23, 1970, now Patent No. 3,716,479. This application Oct. 25, 1972, Ser. No. 300,550  
The portion of the term of the patent subsequent to Feb. 13, 1990, has been disclaimed  
Int. Cl. C10g 23/02

U.S. CL. 208—251 H

9 Claims

### ABSTRACT OF THE DISCLOSURE

This specification discloses a process for the demetalation of hydrocarbon charge stocks containing metal impurities. The process comprises contacting said hydrocarbon charge stock with hydrogen and with a catalyst comprising salt water manganese nodules. These nodules have been previously washed with water having a temperature of at least 125° F. and a total salts content of not more than 1000 parts per million for a time sufficient to increase the accessible surface area of the nodules.

### CROSS REFERENCE TO RELATED APPLICATIONS

This application is a continuation-in-part of our co-pending application Ser. No. 100,931 now U.S. Pat. No. 3,716,479, filed Dec. 23, 1970.

### BACKGROUND OF THE INVENTION

#### Field of the invention

This invention relates to the treatment of a hydrocarbon charge stock and relates more particularly to the treatment of a hydrocarbon charge stock employing a manganese nodule catalyst to effect removal from the hydrocarbon charge stock of organo-metallic compounds.

#### Description of the prior art

U.S. Pat. No. 3,214,236 discloses hydrogenation, desulfurization and denitrogenation as being conversion processes in which manganese nodules are catalytically useful. This patent also discloses that the manganese nodule catalyst can be a source of manganese and other valuable metals after being spent in effecting the desired catalytic conversion.

U.S. Pat. No. 3,509,041 discloses the use of manganese nodules, after pretreatment by base exchange to bond hydrogen ions thereto, in hydrocarbon conversion reactions, specifically cracking, hydrocracking, oxidation, olefin hydrogenation, and olefin isomerization.

U.S. Pat. No. 3,330,096 discloses the use of manganese nodules for removing sulfur compounds from gases.

U.S. Pat. No. 3,471,285 discloses the selective separation of manganese and iron from manganese nodules which also contain cobalt and nickel by reducing the nodules at elevated temperatures and then leaching with an aqueous solution of ammonium sulfate.

### SUMMARY OF THE INVENTION

In accordance with the invention, a hydrocarbon charge stock containing metal impurities is demetalized by contacting the charge stock with hydrogen, in the presence of, as a catalyst, salt water manganese nodules. These salt water manganese nodules have been previous-

## 2

ly washed with water having a temperature of at least 125° F. and a total salts content of not more than 1000 parts per million. The washing is continued for a time sufficient to increase the accessible surface area of the nodules.

### DESCRIPTION OF THE PREFERRED EMBODIMENTS

Various hydrocarbon charge stocks such as crude petroleum oils, topped crudes, heavy vacuum gas oils, shale oils, oils from tar sands, and other heavy hydrocarbon fractions such as residual fractions and distillates contain varying amounts of non-metallic and metallic impurities. The non-metallic impurities include nitrogen, sulfur, and oxygen and these exist in the form of various compounds and are often in relatively large quantities. The most common metallic impurities include iron, nickel, and vanadium. However, other metallic impurities including copper, zinc, and sodium are often found in various hydrocarbon charge stocks and in widely varying amounts. The metallic impurities may occur in several different forms as metal oxides or sulfides which are easily removed by single processing techniques such as by filtration or by water washing. However, the metal contaminants also occur in the form of relatively thermally stable organo-metallic complexes such as metal porphyrins and derivatives thereof along with complexes which are not completely identifiable and which are not so readily removed.

The presence of the metallic impurities in the hydrocarbon charge stocks is a source of difficulty in the processing of the charge stocks. The processing of the charge stock, whether the process is desulfurizing, cracking, reforming, isomerizing, or otherwise, is usually carried out in the presence of a catalyst and the metallic impurities tend to foul and inactivate the catalyst to an extent that may not be reversible. Fouling and inactivation of the catalyst are particularly undesirable where the catalyst is relatively expensive, as, for example, where the active component of the catalyst is platinum. Regardless of the cost of the catalyst, fouling and inactivation add to the cost of the processing of the charge stock and therefore are desirably minimized.

Demetalation of the hydrocarbon charge stock can be effected by thermal processing of the charge stock. However, thermal processing results in conversion of an appreciable portion of the charge stock to coke and the portion of the charge stock converted to coke represents a loss of charge stock that desirably should be converted to a more economically valuable product or products. Moreover, by thermal processing, the metallic impurities tend to deposit in the coke with the result that the coke is less economically desirable than it would be in the absence of the metals.

Demetalation can also be effected by catalytic hydroprocessing of the charge stock. However, catalytic hydroprocessing results in the catalyst becoming fouled and inactivated by deposition of the metals on the catalyst. There is no convenient way of regenerating the catalyst and it ultimately must be discarded. Since these catalysts are relatively expensive, catalytic hydroprocessing to demetalize hydrocarbon charge stocks has suffered from adverse economics.

In our aforementioned copending application, Ser. No. 100,931, there is disclosed a process for demetalation of a hydrocarbon charge stock employing hydrogen in the presence of, as a catalyst, a material derived from the naturally-occurring underwater deposit known as an man-

ganese nodule. As disclosed in the copending application, an economical and effective demetalation of a hydrocarbon charge stock is obtained. Manganese nodules are readily available in large quantities and are relatively inexpensive. Further, material derived from the nodules is capable of effectively removing the metallic impurities from a hydrocarbon charge stock. Thus, whereas the material obtained from the manganese nodules becomes fouled and inactivated by the demetallizing process, the material is obtainable at such low cost that the fouled and inactivated material can be discarded without significant effect on the economics of the demetallizing process.

Manganese nodules, as is known, are naturally-occurring deposits of manganese, along with other metals, including iron, cobalt, nickel, and copper, found on the floors of bodies of water. The body of water may be that of salt water such as in the seas or oceans or may be relatively fresh water such as in lakes. Thus, for example, they are found in abundance on the floor of the Atlantic and Pacific Oceans and on the floor of Lake Michigan. By "salt water manganese nodules," we mean those found on the floor of bodies of salt water such as the Atlantic and Pacific Oceans.

Our present invention is predicated upon our discovery that the catalytic activity of salt water manganese nodules for demetalation, and desulfurization, can be improved by washing the nodules with water. The washing is carried out with water having a temperature of at least 125° F. Further, the water has a total salts content of not more than 1000 parts per million.

The reason why washing of the salt water manganese nodules with water having a temperature of at least 125° F. and a total salts content of not more than 1000 parts per million improves the catalytic activity of the nodules is not thoroughly understood. This washing effects an increase in the accessible surface area of the nodules. By "accessible surface area," we mean the surface area of the nodules which the hydrocarbon charge stock is able to contact. It also effects reduction in the chloride content of the nodules. Whether the increase in the accessible surface area or the decrease in the chloride content, or both, is the essential factor in improving the catalytic properties of the salt water manganese nodules is not known. However, while it is not intended to limit the invention to the consequences of any theory, it is believed that the improvement in the catalytic activity of the nodules is due to the increase in the accessible surface area.

As stated, washing is carried out with water having a temperature of at least 125° F. With this temperature, improvement in the catalytic activity of the salt water manganese nodule is obtained. Higher temperatures, however, are preferred. For example, the temperature of the water employed for washing is preferably about the boiling temperature, namely about 212° F. Still higher temperatures may be employed where the washing is carried out under higher conditions of pressure.

The water employed for washing has a total salts content of less than 1000 parts per million. Satisfactory improvement in the catalytic activity of the nodules is obtained with water having this total salts content. For example, the water may have a total salts content of not more than 500 parts per million. Preferably, fresh water is employed, i.e., potable water. Distilled water may also be employed.

By "washing" is meant contacting the salt water manganese nodules with the water. With contacting, a diffusion of the water into the nodules occurs. Further, a diffusion of a solution of salts out of the nodules occurs. Thus, washing can be effected by immersing the manganese nodules in the wash water. Immersion may be effected one or more times employing new wash water for each immersion. Preferably, in washing, the manganese nodules and the wash water are moved relative to each other. Thus, where washing is effected by immersion, the

wash water may be stirred or otherwise agitated with the manganese nodules being stationary or both the wash water and the manganese nodules may be moved relative to each other by stirring sufficiently vigorously to move the manganese nodules as well as the wash water. The mixture of manganese nodules and wash water may also be tumbled to effect relative movement as by rocking or otherwise effecting oscillating movement of the container holding the manganese nodules and the wash water. Washing may also be effected by passing the water over the manganese nodules as by passing the water through a bed of the nodules. Washing may also be effected by immersing the manganese nodules in the wash water and subjecting the wash water to boiling. A particularly effective way of washing the manganese nodules is by Soxhlet extraction.

The time of washing should be sufficient to effect a significant increase in the accessible surface area of the manganese nodules. By "significant increase" is meant an increase sufficient to effect a measurable improvement in the catalytic activity of the nodules.

The time of washing to effect any desired degree of increase in the accessible surface area of the nodules will depend upon the temperature and the total salt content of the water. It will also depend upon the volume of the wash water relative to the volume of the manganese nodules and the degree of movement of the wash water relative to the nodules. With higher temperatures and lower total salt content, shorter times may be employed. Similarly with greater volumes and greater degree of movement, shorter times may be employed. Generally, any time of washing of at least 5 minutes will increase the accessible surface area of the nodules sufficiently to effect a measurable improvement in the catalytic activity of the nodules.

Prior or subsequent to the washing, the manganese nodules can be crushed and sized to obtain a desired particle size depending upon the type demetalation operation employed, for example, a fixed bed operation, an ebullition operation, or otherwise.

The demetalation reaction is carried out by contacting the hydrocarbon charge stock simultaneously with the catalyst and with hydrogen. The temperatures at which the reaction is carried out can be from about 650° F. to about 850° F. At the higher temperatures, a greater degree of demetalation occurs. However, the temperature employed should not be so high as to effect an undesirable degree of alteration of the charge stock. Preferably, the temperatures employed are in the range of 750-850° F. The pressures at which the reaction is carried out can be from about 100 to about 3000 pounds per square inch gage (p.s.i.g.). Preferably, the pressures employed are in the range of 500-2000 p.s.i.g. Where the reaction is carried out by passing the hydrocarbon charge stock through a bed of the catalyst, the liquid hourly space velocity (LHSV) of the charge stock can be from about 0.2 to 4, preferably 0.5 to 2, volumes of charge stock per volume of catalyst per hour. Hydrogen circulation is at rates of 2000-15,000, preferably 5000-10,000, standard cubic feet of hydrogen per barrel of hydrocarbon charge stock. The hydrocarbon charge stock along with the hydrogen may be passed upwardly through a fixed bed of the catalyst in an upflow reactor or may be passed downwardly through a fixed bed of the catalyst in a downflow trickle-bed reactor. The reaction may also be carried out by passing the charge stock and the hydrogen through an ebullient bed of the catalyst. The reaction may also be carried out by contacting the charge stock, the hydrogen, and the catalyst in a batch reactor.

The process of the invention may be employed for the demetalation of any hydrocarbon charge stock containing organo-metallic compounds. Ordinarily, these will be hydrocarbon charge stocks containing sufficient metal to cause difficulty in the processing, or other subsequent use, of the charge stocks. Other subsequent use of the charge

stocks can include burning of the charge stock as fuel wherein the metals cause corrosion problems. These charge stocks include whole crude petroleum oils, topped crude oils, residual oils, distillate fractions, heavy vacuum gas oils, shale oils, oils from tar sands, and other heavy hydrocarbon oils. Charge stocks derived from Mid-Continent and East Texas crudes contain small amounts of metals. For example, some East Texas crudes contain about 0.1 part per million of vanadium and 2-4 parts per million of nickel. Charge stocks derived from West Texas crudes and foreign crudes, however, can contain larger amounts of metal. Kuwait crude can contain over 32 parts per million of vanadium and over 9 parts per million of nickel while Venezuelan crudes can contain 200-400 parts per million of vanadium and 17 to 59 parts per million of nickel.

The process of the invention can be carried out in conjunction with subsequent steps of processing of the hydrocarbon charge stock. For example, the hydrocarbon charge stock can be subsequently processed for removal of sulfur and/or nitrogen. Further, for example, the hydrocarbon charge stock can be subsequently processed by catalytic cracking.

The following examples will be illustrative of the invention.

#### Example 1

This example will be illustrative of the effect of washing on the catalytic effect of manganese nodules from the Atlantic Ocean.

A sample of manganese nodules obtained from the Blake Plateau in the Atlantic Ocean was crushed. A portion of this material was sieved to 14-30 mesh, U.S. Standard Sieve Series, and was designated Catalyst A. Another portion of the crushed material was washed with boiling water, i.e., at a temperature of 212° F., three times, each wash being of four minutes duration. Washing was effected by suspending the crushed material in a basket and immersing the basket containing the crushed material in boiling distilled water, new water being used for each wash. The washed material was dried and sieved to 14-30 mesh. A portion of this material was designated Catalyst B. The remainder of this washed material was then extracted with distilled water in a Soxhlet extractor for 44 hours. Thereafter, the Soxhlet extracted material was dried and sieved to 14-30 mesh. This latter material was designated Catalyst C.

Each of Catalysts A, B, and C was analyzed for surface area, pore volume, particle density, real density, average pore diameter, and chloride content. These properties are set forth in Table I. In this table, and in the subsequent tables, surface area is given in square meters per gram (m.<sup>2</sup>/g.), pore volume in cubic centimeters per gram (cc./g.), particle density and real density in grams per cubic centimeter (g./cc.), the average pore diameter

in angstrom units (A.), and the chloride content in weight percent (wt. percent).

TABLE I

| Catalyst                           | A     | B     | C     |
|------------------------------------|-------|-------|-------|
| Surface area (m. <sup>2</sup> /g.) | 277   | 296   | 368   |
| Pore volume (cc./g.)               | .388  | .386  | .437  |
| Particle density (g./cc.)          | 1.461 | 1.463 | 1.389 |
| Real density (g./cc.)              | 3.377 | 3.359 | 3.538 |
| Avg. pore diameter (A.)            | 42    | 52    | 48    |
| Chloride content (wt. percent)     | 0.89  | 0.02  | 0.02  |

It will be noted from Table I that washing reduced the chloride content of Catalyst A from 0.89% to 0.02% in the case of both Catalysts B and C. However, it will also be noted that the additional Soxhlet washing received by Catalyst C did not reduce its chloride content below that of Catalyst B. However, the Soxhlet extracts were evaporated to dryness and the recovered material represented removal of about 2% by weight of solids from the nodules. It is believed that these solids removed during the extended Soxhlet washing of the nodules were slightly soluble aluminates and silicates.

The three catalysts were employed in the demetalation of a hydrocarbon charge stock, namely, a Kuwait atmospheric residual oil. This oil had the characteristics given in Table II. In this table, gravity is given in degrees American Petroleum Institute (°API), the amounts of sulfur, nitrogen, carbon and hydrogen and the Conradson Carbon Residue in weight percent (wt. percent), and the amounts of iron (Fe), nickel (Ni), and vanadium (V) in parts per million (p.p.m.).

TABLE II

|                                        |      |
|----------------------------------------|------|
| Gravity (° API)                        | 18.4 |
| Sulfur (wt. percent)                   | 3.89 |
| Nitrogen (wt. percent)                 | 0.19 |
| Conradson Carbon Residue (wt. percent) | 7.23 |
| Carbon (wt. percent)                   | 84.5 |
| Hydrogen (wt. percent)                 | 11.4 |
| Fe (p.p.m.)                            | 4.3  |
| Ni (p.p.m.)                            | 12   |
| V (p.p.m.)                             | 46   |

Demetalation was carried out by passing the oil through a downflow trickle-bed reactor along with hydrogen for over 90 hours. Reaction conditions were as follows:

|                           |                  |
|---------------------------|------------------|
| LHSV                      | 1.0              |
| Temperature               | ° F. 775         |
| Hydrogen circulation rate | s.c.f./b. 10,000 |
| Pressure                  | p.s.i.g. 1000    |

The results are given for each of Catalysts A, B, and C in Tables III, IV, and V, respectively. In these tables, the time on stream is given in hours (hrs.). The desulfurization and demetalation are given as percent (percent) desulfurization and demetalation.

TABLE III.—RESULTS WITH CATALYST A

| Sample                        | 1    | 2    | 3    | 4    | 5    | 6    | 7    | 8    | 9    |
|-------------------------------|------|------|------|------|------|------|------|------|------|
| Time on stream (hrs.)         | 2    | 10.5 | 21   | 33   | 45   | 57   | 69   | 81   | 91   |
| Liquid properties:            |      |      |      |      |      |      |      |      |      |
| Gravity (° API)               | 21.2 | 20.7 | 20.3 | 20.3 | 20.3 | 20.3 | 20.3 | 20.3 | 20.3 |
| Sulfur (wt. percent)          | 3.60 | 3.79 | 3.65 | 3.60 | 3.66 | 3.72 |      |      |      |
| Ni (p.p.m.)                   | 5.2  | 9.9  | 10   | 1 1  | 11   | 11   | 12   | 11   | 11   |
| V (p.p.m.)                    | 16   | 25   | 34   | 35   | 37   | 37   | 38   | 38   | 39   |
| (Ni + V) (p.p.m.)             | 21.2 | 34.9 | 44   | 46   | 48   | 48   | 50   | 49   | 50   |
| Percent desulfurization       | 7.4  | 2.6  | 6.2  | 10.0 | 5.9  | 4.4  |      |      |      |
| Percent demetalation (Ni + V) | 63.4 | 39.8 | 24.1 | 20.7 | 17.2 | 17.2 | 13.8 | 15.5 | 13.8 |

TABLE IV.—RESULTS WITH CATALYST B

| Sample                        | 1    | 2    | 3    | 4    | 5    | 6    | 7    | 8    | 9    |
|-------------------------------|------|------|------|------|------|------|------|------|------|
| Time on stream (hrs.)         | 2    | 10.5 | 21   | 33   | 45   | 57   | 69   | 81   | 90.5 |
| Liquid properties:            |      |      |      |      |      |      |      |      |      |
| Gravity (° API)               | 21.7 | 21.2 | 20.7 | 20.7 | 20.7 | 20.7 | 20.7 | 20.7 | 20.7 |
| Sulfur (wt. percent)          | 2.33 | 2.80 | 3.34 |      | 3.36 | 3.40 | 3.45 | 3.53 | 3.48 |
| Ni (p.p.m.)                   | 3.7  | 7.4  | 8.7  | 9.8  | 10   | 11   | 11   | 11   | 11   |
| V (p.p.m.)                    | 9.4  | 20   | 26   | 28   | 28   | 29   | 29   | 29   | 29   |
| (Ni + V) (p.p.m.)             | 14.1 | 27.4 | 34.7 | 35.8 | 38   | 39   | 40   | 40   | 40   |
| Percent desulfurization       | 40.1 | 28.0 | 14.1 |      | 13.6 | 12.6 | 11.3 | 9.3  | 10.5 |
| Percent demetalation (Ni + V) | 75.7 | 52.8 | 40.2 | 38.3 | 34.5 | 32.8 | 31.0 | 31.0 | 31.0 |

TABLE V.—RESULTS WITH CATALYST C

| Sample                        | 1    | 2    | 3    | 4    | 5    | 6    | 7    | 8    | 9    |
|-------------------------------|------|------|------|------|------|------|------|------|------|
| Time on stream (hrs.)         | 2    | 10.5 | 21   | 33   | 45   | 57   | 69   | 81   | 91   |
| Liquid properties:            |      |      |      |      |      |      |      |      |      |
| Gravity (° API)               | 28.2 | 21.3 | 21.2 | 21.2 | 21.2 | 21.2 | 21.1 | 21.1 | 21.1 |
| Sulfur (wt. percent)          | 2.46 | 2.96 | 3.09 | 3.10 | 3.13 | 3.12 | 3.16 | 3.07 | 3.06 |
| Ni (p.p.m.)                   | 2.7  | 6.5  | 7.9  | 8.4  | 8.8  | 9.4  | 9.8  | 9.8  | 9.8  |
| V (p.p.m.)                    | 5.9  | 13   | 18   | 21   | 22   | 23   | 24   | 24   | 24   |
| (Ni + V) (p.p.m.)             | 8.6  | 19.5 | 25.9 | 29.4 | 30.8 | 32.4 | 33.8 | 33.8 | 33.8 |
| Percent desulfurization       | 36.8 | 23.9 | 20.5 | 20.3 | 19.5 | 19.8 | 18.8 | 21.1 | 21.3 |
| Percent demetalation (Ni + V) | 85.2 | 66.3 | 55.3 | 49.3 | 46.9 | 44.1 | 41.7 | 41.7 | 41.7 |

It will be observed from Tables III, IV, and V that the demetalation activity of Catalyst B was greater than that of Catalyst A and that of Catalyst C greater than that of Catalyst B. The average demetalation for Cat-

The two catalysts were employed for the demetalation of the same residual oil and at the same reaction conditions described in Example 1. The results are given in Tables VII and VIII.

TABLE VII.—RESULTS WITH CATALYST D

| Sample                        | 1    | 2    | 3    | 4    | 5    | 6    | 7    | 8    | 9    |
|-------------------------------|------|------|------|------|------|------|------|------|------|
| Time on stream (hrs.)         | 2    | 10.5 | 21   | 33   | 45   | 57   | 69   | 81   | 91   |
| Liquid properties:            |      |      |      |      |      |      |      |      |      |
| Gravity (° API)               | 21.2 | 20.9 | 20.9 | 20.9 | 20.9 | 20.9 | 20.9 | 20.9 | 20.9 |
| Sulfur (wt. percent)          | 3.04 | 3.38 | 3.45 | 3.43 | 3.38 | 3.44 | 3.51 | 3.51 | 3.54 |
| Ni (p.p.m.)                   | 5.4  | 8.8  | 9.8  | 10   | 10   | 10   | 10   | 10   | 11   |
| V (p.p.m.)                    | 9.9  | 16   | 20.0 | 20   | 20   | 20   | 20   | 21   | 22   |
| (Ni + V) (p.p.m.)             | 15.3 | 24.8 | 29.8 | 30.0 | 30.0 | 30.0 | 30.0 | 31.0 | 33.0 |
| Percent desulfurization       | 21.9 | 13.1 | 11.3 | 11.8 | 13.1 | 11.6 | 9.8  | 9.8  | 9.0  |
| Percent demetalation (Ni + V) | 73.6 | 57.2 | 48.6 | 48.3 | 48.3 | 48.3 | 48.3 | 46.6 | 43.1 |

TABLE VIII.—RESULTS WITH CATALYST E

| Sample                        | 1    | 2    | 3    | 4    | 5    | 6    | 7    | 8    | 9    |
|-------------------------------|------|------|------|------|------|------|------|------|------|
| Time on stream (hrs.)         | 2    | 10.5 | 21   | 33   | 45   | 57   | 69   | 81   | 91   |
| Liquid properties:            |      |      |      |      |      |      |      |      |      |
| Gravity (° API)               | 24.2 | 21.6 | 20.7 | 21.3 | 21.1 | 21.1 | 20.8 | 20.8 | 20.8 |
| Sulfur (wt. percent)          | 2.26 | 2.91 | 3.02 | 2.95 | 2.98 | 3.01 | 3.02 | 2.99 | 2.95 |
| Ni (p.p.m.)                   | 2.5  | 6.9  | 8.0  | 8.3  | 9.5  | 9.7  | 9.3  | 9.8  | 9.4  |
| V (p.p.m.)                    | 2.7  | 9.8  | 13.0 | 13.0 | 14.8 | 16.4 | 16.7 | 19.3 | 19.2 |
| (Ni + V) (p.p.m.)             | 5.2  | 16.7 | 21.0 | 21.3 | 24.3 | 26.1 | 26.0 | 29.1 | 28.6 |
| Percent desulfurization       | 41.9 | 25.2 | 22.4 | 24.2 | 23.4 | 22.6 | 22.4 | 23.1 | 24.2 |
| Percent demetalation (Ni + V) | 91.0 | 71.2 | 63.8 | 63.3 | 58.1 | 55.0 | 55.2 | 49.8 | 50.7 |

alysts A, B, and C was 22.8%, 38.7%, and 50.3%, respectively, indicating the effectiveness of the washing applied to Catalyst B and the additional effectiveness of the Soxhlet washing applied to Catalyst C. Stated otherwise, as indicated in Tables III, IV, and V, the depth of washing has a major influence on the demetalation activity of the nodules. It will also be observed from Tables III, IV, and V that washing also significantly improved the desulfurization activity of the nodules.

#### Example 2

This example will illustrate the effect of washing on the catalytic effect of manganese nodules from the Pacific Ocean.

Manganese nodules obtained from the bottom of the Pacific Ocean were crushed and were washed three times with boiling distilled water, the washing being carried out in the manner and for the times described in Example 1. The nodules were then dried and sieved to 14-30 mesh. A portion of the dried material was designated Catalyst D. The remainder of the dried material was extracted in a Soxhlet extractor with distilled water for 71 hours. The extracted material was dried and resieved to 14-30 mesh. This material was designated Catalyst E. The properties and chloride content were determined and are given in Table VI.

TABLE VI

| Catalyst                           | D     | E     |
|------------------------------------|-------|-------|
| Surface area (m. <sup>2</sup> /g.) | 210   | 411   |
| Pore volume (cc./g.)               | 0.406 | 0.468 |
| Particle density (g./cc.)          | 1.45  | 1.37  |
| Real density (g./cc.)              | 3.59  | 3.78  |
| Avg. pore diameter (A.)            | 78    | 46    |
| Chloride content (wt. percent)     | 0.50  | <0.01 |

It will be noted from Tables VII and VIII that washing of the nodules improved their catalytic activity for demetalation. It will also be noted that washing of the nodules approximately doubled their activity for desulfurization.

We claim:

1. A process for the demetalation of a hydrocarbon charge stock containing metal impurities comprising contacting said hydrocarbon charge stock with hydrogen and with a catalyst comprising salt water manganese nodules which have been washed with water having a temperature of at least 125° F. and a total salts content of not more than 1000 parts per million for a time sufficient to increase the accessible surface area of said nodules.
2. The process of claim 1 wherein said manganese nodules are nodules from the Atlantic Ocean.
3. The process of claim 1 wherein said manganese nodules are nodules from the Pacific Ocean.
4. The process of claim 1 wherein said nodules are washed with water having a temperature of about 212° F.
5. The process of claim 1 wherein said nodules have been washed by Soxhlet extraction.
6. The process of claim 1 wherein said nodules have been washed with water having a total salts content of not more than 500 parts per million.
7. The process of claim 1 wherein said nodules have been washed with fresh water.
8. The process of claim 1 wherein said nodules have been washed with distilled water.

3,813,331

9

9. The process of claim 1 wherein said nodules have  
been washed for at least 5 minutes.

10

3,471,285 11/1969 Rolf ----- 75-115  
3,509,041 4/1970 Miale ----- 208-119

References Cited

UNITED STATES PATENTS

3,716,479 2/1973 Weisz et al. ----- 208-211  
3,214,236 11/1965 Weisz et al. ----- 252-471

DELBERT E. GANTZ, Primary Examiner

5 J. M. NELSON, Assistant Examiner

U.S. Cl. X.R.

208-211; 252-454

UNITED STATES PATENT OFFICE  
CERTIFICATE OF CORRECTION

Patent No. 3,813,331 Dated May 28, 1974

Inventor(s) Paul B. Weisz and Anthony J. Silvestri

It is certified that error appears in the above-identified patent and that said Letters Patent are hereby corrected as shown below:

Column 2, line 67, "as an" should read --as a--.

Column 4, line 38, after "type" insert --of--;  
line 46, "temperature" should read --temperatures--.

Column 7, Table VI, last line, "<00.1" should read

-- <0.01--.

Column 9, and column 10, two of the references cited should  
read: 3,214,236 10/1965 Weisz 252-471  
3,471,285 10/1969 Rolf 75-115

Signed and sealed this 1st day of October 1974.

(SEAL)

Attest:

McCORY M. GIBSON JR.  
Attesting Officer

C. MARSHALL DANN  
Commissioner of Patents